

# United States Patent Office

2,739,915

Patented Mar. 27, 1956

1  
2,739,915

## MULTIPLE ACTION LUBRICATING COMPOSITION

Ludwig Karl Schuster, Philadelphia, and Harvey Aurand Whitenight, Norristown, Pa.

No Drawing. Application July 20, 1950,  
Serial No. 175,028

7 Claims. (Cl. 148—6.15)

This invention relates to improved compositions for the lubrication of metal for the purpose of conducting mechanical forming processes such as, drawing, stamping, cutting, ironing, upsetting, extrusion, rolling, and similar metal forming processes where boundary lubrication is necessary to reduce the high friction and to insure separation of work and tools. The invention relates particularly to the preparation and use of lubricant compositions wherein a stable organic lubricant phase is present with a chemical substance having an inorganic cation and capable of reacting chemically with the surface of the work piece in the presence of water to deposit a coating selected from the group consisting of metal coatings, insoluble inorganic salt coatings and insoluble organo-inorganic salt coatings. Base metals with which the invention is useful are those substantially of ferritic crystal structure.

The usefulness of organic polar lubricants in particular has been well established in such metal forming processes. The general use of fatty acids, fatty soaps, and fatty oils, such as stearic acid, tallow, lard oil, palm oil, alone or oftentimes emulsified in water is sufficient proof of the utility of such materials. However, in many metal forming processes, unit pressures occur which rupture the lubricant film formed by such organic polar lubricants alone. The addition of inert fillers and pigments, such as chalk and mica, to such organic lubricants provides better separation of the metal being formed from the forming tools and/or dies. This method of improving the utility of organic polar lubricants is likewise in general use.

Still another method of providing improved lubricant films for such metal forming processes is to pre-deposit on the metal surface a tenacious inorganic coating. Oxides of the base metal, such as rust, alone or together, with inorganic materials such as lime, borax, silicates, are types of such coatings. Likewise, metallic phosphate, oxalate, sulphite and similar coatings have utility. Coatings of the more ductile metals, such as copper, lead, and tin are widely used.

A primary object of the invention is to provide a relatively stable multiple action lubricating composition for application to a steel work piece substantially of ferritic crystal structure, to provide on the work piece both a chemically deposited coating capable of providing a high degree of separation of work and tool during cold working of the piece and an organic friction reducing substance, said composition comprising a coating constituent including a substance having an inorganic cation and capable of reacting chemically with the surface of the work piece in the presence of water to deposit a coating selected from the group consisting of metal coatings, insoluble inorganic salt coatings and insoluble organo-inorganic salt coatings, and an organic lubricant constituent which includes a cationic surface active compound.

A further object of the invention is to provide a multiple action lubricating composition as described in the preceding object, in which the cationic surface active compound is selected from the group consisting of simple acid

2  
salts of nitrogen, quaternary salts of nitrogen and heterocyclic nitrogen compounds, where the compound includes a long chain hydrophobe radical.

Another object of the invention is to provide a relatively stable multiple action lubricating composition for application to a steel work piece substantially of ferritic crystal structure, to provide on the work piece both a chemically deposited coating capable of providing a high degree of separation of work and tool during cold working of the piece and an organic friction reducing substance, said composition comprising an acidic coating constituent including a substance having an inorganic cation and an anion capable of reacting chemically with the surface of the work piece in the presence of water to form thereon a coating selected from the group consisting of metal coatings, insoluble inorganic salt coatings and insoluble organo-inorganic salt coatings, and an organic lubricant constituent which includes a cationic surface active compound.

Other objects will be apparent from a study of this specification and the appended claims.

In many metal forming operations the best results have been obtained by the use of tenacious inorganic coatings in conjunction with an organic lubricant. As these coatings often require the use of acidic plating or coating baths, it has been necessary that they be applied separately from the organic lubricants, with intermediate rinsing advisable, and usually very necessary. The separate application of the coating materials and the lubricating materials has until now been considered necessary for the reason that it was thought impossible to provide stable and uniform compositions for supplying both by application of a single composition.

The practical desirability of a multiple action lubricant which will deposit by a single application both the tenacious coating and the organic lubricant should be apparent. Not only does such a multiple action lubricant film have many practical advantages, in saving application steps and making the process economical and trouble free, but it provides a more uniform lubricant film because of the simultaneous application of the coating and lubricant substances.

To achieve homogeneous multiple action lubricant compositions both prior to and after application to the metal surface, cationic surface active agents have been found 45 the most desirable as the organic phase, or as a necessary component of that phase. This feature is an important part of the present invention.

Of the cation active materials investigated, whether used alone as lubricants, or as emulsifiers for other organic lubricants, we have found most suitable the simple acid salts and quaternary salts of nitrogen, where the nitrogen may be joined to the hydrophobe directly, as in an amine, or by means of an intermediate linkage, as in an amide. By a hydrophobe is meant the accepted colloid significance of this term—straight chain, branched chain, aromatic, or cyclic radicals, their combined forms or a plurality of these groups where the total number of carbon atoms exceeds 10. The invention is most useful where the number of carbon atoms is from 16 to 18, but hydrophobe radicals can be used where the number of carbon atoms exceeds 10.

Less effective, but nevertheless suitable are the heterocyclic nitrogen compounds as well as the non-nitrogenous cation-active sulfonium and phosphonium types, 65 Members of other classifications of cationic agents are apparently suitable, that is, members which may be classified as guanidine, hydrazine, amine oxide, arsonium, and amphotolytic types, the latter having both an acidic and basic group in the same molecule.

The use of these cation active substances as a component provides a multiple action lubricant which meets for the first time the following requirements:

1. Homogeneous dispersions of the lubricant in water over a wide range of temperatures and concentrations.

2. The ability to prepare very concentrated combinations of the organic and inorganic components, such combinations being suitable for marketing, storage, and shipment as "one package" lubricants.

3. More certain and better lubrication of metals during forming operations than now provided in many cases by separate applications of inorganic coatings and organic lubricants. Some of the cationic substances have in themselves surprisingly excellent friction reducing properties and can be used as the entire organic phase.

4. Ease of application and use provided by single lubricant application.

5. The ability to form inorganic coatings of better quality on soiled metal surfaces by virtue of the detergency provided by the organic phase, as well as the levelling action of the cation agents in the presence of acid media and strong electrolytes.

6. Protection of the coated metal and metal forming equipment against atmosphere corrosion by the immediate and simultaneous deposition of the organic phase.

Anionic surface-active agents, for which the active hydrophobe carries a negative charge, are in the main precipitated by the electropositive character of strongly acidic media and solutions of heavy metal salts. A selected few have been suggested as wetting agents for use in phosphate baths, but for those of possible merit the hydrophilic/hydrophobic balance is so high that they are useless as either lubricants or emulsifiers for lubricant materials. Since the anionic agents are almost predominantly organic sulfates or sulfonates, they contain inorganic sulfates as residues of manufacture unless uneconomical processes are used for purification. The inorganic sulfates, obviously, promote corrosion.

The non-ionic agents exhibit water solubility and emulsifying characteristics by virtue of their ability to solvate by hydrogen bonding. Since these compounds are not dissociated in water media, they remain more or less colloidally stable in the presence of solutions of mineral acid and metallic salts. However, they do not provide dispersions of such a high degree of stability as do the cationics, and the non-ionics usually provide dispersions of increasing instability as temperatures increase. This latter characteristic would make difficult, if not impossible, proper application in most instances.

Those members of the non-ionic group which are esters, of course, would undergo decomposition into their constituent acidic and alcohol groups in the presence of dilute mineral acid. Solubility of the non-ionics over a wide range of acidity and basicity is a disadvantage in this type of application, as such an organic phase does not enhance the corrosion resistance of the coated metal. Likewise, the progressive insolubility of the cationics when in contact with metal provides a means of precipitating the organic phase in intimate contact with the inorganic; this phenomenon does not occur when non-ionics are employed. Nevertheless, we have found that some non-ionic substances are valuable adjuncts as blending agents in some compositions where the cationic type lubricant is not miscible with the inorganic coating concentrate as prepared for subsequent dilution. On the basis of emulsion stability, we have also found in some cases that each displays a synergism for the other, whereby emulsions are obtained which are more stable than would be possible for either alone.

The coating part of the lubricant can consist of:

A. One or more substances having an inorganic cation, which substances in the presence of water form a film on a metal surface of an inorganic, insoluble salt, the cation of which is substantially or entirely provided by the metal surface so treated. Such salt films are, for instance, iron oxide, iron sulphide, and iron phosphate. Oxide films can be formed by the use of solutions containing oxidants, such as chromates, nitrites, nitrates, chlorates, permanga-

nates. More suitable oxide coatings can be produced using such oxidants mentioned above in the presence of relatively weak acids, such as phosphoric or hydrosilicofluoric acid. Phosphate coatings can be formed using, for example, solutions of mono- or di-ammonium phosphate, potassium phosphate, or sodium phosphate.

B. One or more substances, which, in the presence of water, form a film on a metal surface of an insoluble metal organic salt, the cation of which is provided by the metal surface so treated. Such a salt film is an oxalate. Oxalate coatings can be produced using dilute solutions of oxalic acid or acid oxalates.

C. One or more substances, the cation of which is inorganic, which, in the presence of water forms on a metal surface a film of an insoluble salt, the cation of which is partly or entirely foreign to the metal surface. Typical representatives of this group are the phosphate coatings which can consist of insoluble metal phosphates such as zinc, iron, manganese, cadmium, etc. Phosphate coatings can be formed by the use of acid solutions of manganese or zinc phosphate, or mixtures of zinc, or manganese, and ferrous phosphate. Other acid phosphates may be employed. The formation of the phosphate coating can be accelerated by the addition of metals as salts which are more electropositive than the metal to be coated. Such accelerators are copper, silver, nickel, cobalt salts. Oxidizing agents such as nitrites, nitrates, chlorates may also be incorporated. Organic oxidants such as nitro compounds may also be used.

D. One or more substances capable of producing a metal coating, a typical representative of which is copper. Very adherent copper coatings can be formed using acid solutions of copper sulphate or formate. The addition of strong electrolytes, such as zinc sulphate, to the above solution, further improves the copper coating formed. It can be seen readily, from an inspection of the type of coating substances mentioned above, that one has a wide range of choice the type of coating material as long as the material has an inorganic cation.

In general, the amount of organic lubricant should not be less than 5% of the inorganic component. In the examples which follow, and in the general practice of the invention, the presence of organic lubricant in an amount greater than that required to reach peak efficiency for the combined lubricant does not, in general, have a detrimental effect during metal forming operation, although such practice is not justified on the basis of economy. In many forming operations, excessive organic lubricant will be removed by the pressure exerted between work and tools. Thus, in wire and tube drawing, for example, a portion of the organic lubricant may be lost by removal at the first die pass.

The upper effective limit of concentration of the organic lubricant is controlled somewhat by the resulting physical state of the bath. If the concentration of the organic components becomes so high that the coating bath becomes viscous or gelatinous, and if such baths cannot be thinned by additives (solvents, for example), the rate of deposition of the coating being deposited is inhibited. Increase in the viscosity of the bath decreases the mobility of its components, and as a result the metal/liquid interface may not be maintained at a sufficiently high level of soluble inorganic salts by replacement of the bath proper as coating is being formed on the metal surface. Most of the lubricants useful in the invention lend themselves in varying degrees to thinning with solvents.

In selecting the amount of organic lubricant, a rough method is to set the amount of organic lubricant as the difference between the entirety and the amount of the inorganic salts with the water required for the solution of the inorganic salts.

There are several suitable methods of preparing a multiple action lubricant as described herein. In some cases, the coating and lubricating components may be combined directly. Another suitable method is to prepare the coat-

ing part and the lubricant part separately, and then combine them into the finished multiple action lubricant. With respect to water content, the multiple action lubricant may be prepared in highly concentrated form, or in more diluted form, as where limited solubility or compatibility of the constituents exists.

The mode of application of the multiple action lubricant product is not critical and is generally dictated to a great extent by the type and shape of metal being formed.

While not restricted to any particular method of application it is in most cases conveniently applied by immersion, either at room or elevated temperatures. Its application at elevated temperatures is preferable.

The following compositions will serve to exemplify the invention, although as has been explained above, they do not exhaust the possible variations which may be employed within the scope of the invention. In these examples, the proportions are by weight.

#### Example 1

13% of an amide phosphate having the following composition:

72% of an organic amide lubricant having the following molecular composition: 25

1 mole glycerine mono-fatty acid ester



2 moles fatty amide



14.4% of Emulphor ON (derivative of polyethylene glycol, a condensation product of ethylene oxide and an organic acid supplied by General Dyestuffs Corp. as set forth in Surface Active Agents by Young and Coons, Chemical Publishing Co., 1945.)

13.6% of phosphoric acid (70%  $\text{H}_3\text{PO}_4$ )

87% of a zinc sulfite depositing solution containing:

9% zinc sulphate ( $\text{ZnSO}_4 \cdot 7\text{H}_2\text{O}$ )

3% sodium meta bisulfite ( $\text{Na}_2\text{S}_2\text{O}_5$ )

88%  $\text{H}_2\text{O}$

The amide phosphate was added to the inorganic solution.

The treatment of a steel workpiece with the composition of this example produces a zinc sulfite coating on the piece and also organic lubricant is provided by this treatment.

#### Example 2

13% of an amide phosphate having the following composition:

60.6% of the organic amide lubricant described in Example 1.

12.1% of Emulphor ON

27.3% of phosphoric acid (70%  $\text{H}_3\text{PO}_4$ )

87% of a ferrous oxalate depositing solution containing:

2% oxalic acid ( $\text{COOH})_2 \cdot 2\text{H}_2\text{O}$

1% ferric chloride ( $\text{FeCl}_3 \cdot 6\text{H}_2\text{O}$ )

97%  $\text{H}_2\text{O}$

\* Where  $\text{RCO}-$  and



each represent the acyl radicals of mixed saturated and mono-unsaturated fatty acids of 16 and 18 carbon atoms.

The amide phosphate was added to the inorganic solution.

A ferrous oxalate coating and an organic lubricant is provided on a workpiece treated according to this example.

#### Example 3

20% of N - ethanol - N - (N' - diethanolaminoethyl) stearamide<sup>1</sup>



12% tallow

4% Emulphor ON

6.3% phosphoric acid (70%  $\text{H}_3\text{PO}_4$ )

30% of a primary sodium phosphate solution containing 520 gms.  $\text{NaH}_2\text{PO}_4 \cdot 1$ .

27.7% water

Treatment of a steel workpiece according to this example provides an iron phosphate coating and an organic lubricant.

#### Example 4

21.6% of the organic amide lubricant described in Example 1

96% of phosphoric acid (70%  $\text{H}_3\text{PO}_4$ )

18.8% of an acid zinc phosphate solution containing 178 gms. zinc/l. and 1200 gms. of phosphoric acid (70%  $\text{H}_3\text{PO}_4$ )/liter

50.0% water

Treatment according to this example provides a zinc phosphate coating and an organic lubricant.

#### Example 5

20% of 1-hydroxyethyl-2-heptadecenyl glyoxalidine having the following structural formula:



11.2% phosphoric acid (70%)

18.8% of the acid zinc phosphate solution of Example 4

50% water

This example provides a zinc phosphate coating and an organic lubricant.

#### Example 6

22% primary ammonium phosphate

41%  $\text{H}_2\text{O}$

4% phosphoric acid (70%)

25% diethanol stearamide

8% "Ethomeen" (Armour & Co.)



Treatment according to this example provides an iron phosphate coating and an organic lubricant.

#### Example 7

46.5% of an organic amide lubricant having the following molecular composition:

1 mole glycerine di-fatty acid ester,



<sup>1</sup>This compound is a condensation product formed by the reaction of one mole of stearic acid with two moles diethanolamine at a temperature above 150° C. with loss of water of reaction and a drop in acidity (stearic) to below 5%. Lauric acid can be used in place of stearic acid, the resulting product being more soluble.

and 1 mole fatty amide having the structural formula:

$$\text{RC}-\text{NH}-\text{CH}(\text{CH}_3)-\text{NH}-\text{CH}(\text{CH}_3)-\text{NH}_2$$

where RCO— is the acyl radical of a fatty acid having 16 to 18 carbon atoms.

9.3% Emulphor ON  
16.3% of phosphoric acid (70%  $\text{H}_3\text{PO}_4$ )  
27.9% of the acid zinc phosphate solution described in Example 4.

This example provides a zinc phosphate coating and an organic lubricant.

*Example 8*

25.4% of the organic amide lubricant described in Example 7

25.4% of prime lard oil

10.2% Emulphor ON

8.8% of phosphoric acid (70%  $\text{H}_3\text{PO}_4$ )  
30.2% of the acid zinc phosphate solution described in Example 4.

This example produces a zinc phosphate coating and an organic lubricant.

*Example 9*

51.5% of the organic amide lubricant described in Example 4

10.3% Emulphor ON

7.2% of phosphoric acid (70%  $\text{H}_3\text{PO}_4$ )

31.0% of an acid zinc phosphate solution containing 230 gms. zinc/liter and 1200 gms phosphoric acid (70%  $\text{H}_3\text{PO}_4$ )/liter

This example provides a zinc phosphate coating and an organic lubricant.

*Example 10*

51.5% of the organic amide lubricant described in Example 7

10.3% Emulphor ON

7.2% of phosphoric acid (70%  $\text{H}_3\text{PO}_4$ )

31.0% of an acid zinc phosphate solution containing 230 gms. zinc/liter, 1200 gms. phosphoric acid (70%  $\text{H}_3\text{PO}_4$ )/liter and 5.7 gms. copper/l. as  $\text{CuCl}_2 \cdot 2\text{H}_2\text{O}$

This example provides a zinc phosphate coating and an organic lubricant.

*Example 11*

25.5% of N,N-diethanol-stearamide having the structural formula:



9.0% of phosphoric acid (70%  $\text{H}_3\text{PO}_4$ )  
15.5% of the acid zinc phosphate solution as described in Example 9.  
50.0% water

This example provides a zinc phosphate coating and an organic lubricant.

*Example 12*

7.0% oleic acid

3.0% stearic acid

16.5% of the amide lubricant described in Example 1

25.0% of the amide lubricant described in Example 7

10.3% Emulphor ON

7.2% phosphoric acid (70%  $\text{H}_3\text{PO}_4$ )

31.0% of the acid zinc phosphate solution described in Example 9.

\* Where  $\text{RCO}-$  and

$\text{RCO}-$  each represent the acyl radicals of mixed saturated and mono-unsaturated fatty acids of 16 and 18 carbon atoms.

This example produces a zinc phosphate coating and an organic lubricant.

*Example 13*

5 25.5% stearoyl-diethanol polyethylene glycol ammonium chloride having the following structural formula (dissociated):



2.0% phosphoric acid (70%  $\text{H}_3\text{PO}_4$ )

15.5% of the acid zinc phosphate solution described in Example 9

15 57.0% water.

This example provides a zinc phosphate coating and an organic lubricant.

*Example 14*

20 48.9% of the organic amide lubricant described in Example 1

9.8% Emulphor ON

29.3% of an acid zinc phosphate-nitrate solution containing:

183 gms. zinc/l.

5 gms. nickel/l.

410 gms. phosphoric acid (70%  $\text{H}_3\text{PO}_4$ )/liter

390 gms. nitric acid (60%  $\text{HNO}_3$ )/liter

12.0% of phosphoric acid (70%  $\text{H}_3\text{PO}_4$ )

This example provides a zinc phosphate coating and an organic lubricant.

*Example 15*

35 13% of an amide phosphate as described in Example 1

87% of an acid copper sulphate solution containing:

1.5% copper sulfate ( $\text{CuSO}_4 \cdot 5\text{H}_2\text{O}$ )

2.0% zinc sulfate ( $\text{ZnSO}_4 \cdot 7\text{H}_2\text{O}$ )

5.0% sulphuric acid ( $\text{H}_2\text{SO}_4$  conc.)

The amide phosphate was added to the inorganic solution.

This example provides a metallic copper coating and an organic lubricant.

*Example 16*

30% amide sulfate



50 18.8% of the acid zinc phosphate solution of Example 4

51.2% water

where R is as stated in the other examples.

55. This example provides a zinc phosphate coating and an organic lubricant.

In general, the compound



60 may be used in any example in place of



65 with an increase in the phosphoric acid component.

As illustrated in Examples 3 and 8, various natural fats and oils commonly used for lubrication in metal working processes, such as tallow and lard oil, may be included in the lubricating compositions of the present invention.

The above compositions gave excellent results as metal forming lubricants. A variety of application methods were employed with various water dilutions. Best results were obtained with high concentrations, but economical, satisfactory operation was obtained with solutions con-

taining 80-90% water applied to the metal by immersion at 180-190° F. for 15 minutes.

In the practice of the invention, as shown for example in the working examples set forth herein, the amines, amides and other nitrogenous compounds are cationic only when in the form of salts, and the extra amounts of acid used in these examples, over and above the acid used in the coating part of the composition, serves to convert the organic compounds to salts such as



The "X" designates the anion furnished by the acid used with the organic compounds. For convenience, the claims refer to the organic compounds in their original form before conversion to salts.

Anyone skilled in the art will readily recognize that modification is possible in the products specifically disclosed herein without departing from the essential features or inventive concept of the present invention.

We claim:

1. A relatively stable multiple action lubricating composition for application to a steel work piece substantially of ferritic crystal structure, to provide on the work piece both a chemically deposited coating capable of providing a high degree of separation of work and tool during cold working of the piece and an organic friction reducing substance, said composition comprising:

21.6% of an organic amide lubricant having the following molecular composition:

1 mole glycerine mono-fatty acid ester,  
 $\text{RCOOCH}_2-\text{CHOH}-\text{CH}_2\text{OH}$

2 moles fatty amide,



9.6% of phosphoric acid (70%  $\text{H}_3\text{PO}_4$ ),

18.8% of an acid zinc phosphate solution containing 178 grams zinc/liter and 1200 grams of phosphoric acid (70%  $\text{H}_3\text{PO}_4$ )/liter,

50.0%  $\text{H}_2\text{O}$ ,

where  $\text{RCO}-$  and



each represent the acyl radicals of mixed saturated and mono-unsaturated fatty acids of 16 and 18 carbon atoms.

70

75 7.2% phosphoric acid (70%  $\text{H}_3\text{PO}_4$ )

2. A relatively stable multiple action lubricating composition for application to a steel work piece substantially of ferritic crystal structure, to provide on the work piece both a chemically deposited coating capable of providing a high degree of separation of work and tool during cold working of the piece and an organic friction reducing substance, said composition consisting of:

46.5% of an organic amide lubricant having the following molecular composition:

1 mole glycerine di-fatty acid ester,



1 mole fatty amide



9.3% condensation product of ethylene oxide and an organic acid

16.3% phosphoric acid (70%  $\text{H}_3\text{PO}_4$ )

20 27.9% of an acid zinc phosphate solution containing 178 grams zinc/liter and 1200 grams phosphoric acid (70%  $\text{H}_3\text{PO}_4$ )/liter,

where  $\text{RCO}-$  and



each represent the acyl radicals of mixed saturated and mono-unsaturated fatty acids of 16 and 18 carbon atoms.

30 3. A relatively stable multiple action lubricating composition for application to a steel work piece substantially of ferritic crystal structure, to provide on the work piece both a chemically deposited coating capable of providing a high degree of separation of work and tool during said working of the piece and an organic friction reducing substance, said composition consisting of:

25.4% of an organic amide lubricant having the following molecular composition:

1 mole glycerine di-fatty acid ester,



1 mole fatty amide



45 25.4% prime lard oil

10.2% condensation of ethylene oxide and an organic acid

8.8% phosphoric acid (70%  $\text{H}_3\text{PO}_4$ )

30.2% of an acid zinc phosphate solution containing 178 grams zinc/liter and 1200 grams phosphoric acid (70%  $\text{H}_3\text{PO}_4$ )/liter,

where  $\text{RCO}-$  and



55 each represent the acyl radicals of mixed saturated and mono-unsaturated fatty acids of 16 and 18 carbon atoms.

4. A relatively stable multiple action lubricating composition for application to a steel work piece substantially of ferritic crystal structure, to provide on the work piece both a chemically deposited coating capable of providing a high degree of separation of work and tool during said working of the piece and an organic friction reducing substance, said composition consisting of:

60 51.5% of an organic amide lubricant having the following molecular composition:

1 mole glycerine mono-fatty acid ester,



2 moles fatty amide,



10.3% condensation product of ethylene oxide and an organic acid

## 11

31.0% of an acid zinc phosphate solution containing 230 grams zinc/liter and 1200 grams phosphoric acid (70% H<sub>3</sub>PO<sub>4</sub>)/liter,

where RCO— and



each represent the acyl radicals of mixed saturated and mono-unsaturated fatty acids of 16 and 18 carbon atoms.

5. A relatively stable multiple action lubricating composition for application to a steel work piece substantially of ferritic crystal structure, to provide on the work piece both a chemically deposited coating capable of providing a high degree of separation of work and tool during said working of the piece and an organic friction reducing substance, said composition consisting of:

51.5% of an organic amide lubricant having the following molecular composition:

1 mole glycerine di-fatty acid ester,



1 mole fatty amide



10.3% condensation product of ethylene oxide and an organic acid

7.2% phosphoric acid (70% H<sub>3</sub>PO<sub>4</sub>)

31.0% of an acid zinc phosphate solution containing 230 grams zinc/liter, 1200 grams phosphoric acid (70% H<sub>3</sub>PO<sub>4</sub>)/liter, and 5.7 grams Cu (as CuCl<sub>2</sub>—2H<sub>2</sub>O)/liter,

where RCO— and



each represent the acyl radicals of mixed saturated and mono-unsaturated fatty acids of 16 and 18 carbon atoms.

6. A relatively stable multiple action lubricating composition for application to a steel work piece substantially of ferritic crystal structure, to provide on the work piece both a chemically deposited coating capable of providing a high degree of separation of work and tool during said working of the piece and an organic friction reducing substance, said composition consisting of:

25.5% of N,N-diethanol-stearamide,



9.0% phosphoric acid (70% H<sub>3</sub>PO<sub>4</sub>),

15.5% of an acid zinc phosphate solution 230 grams 55 zinc/liter and 1200 grams phosphoric acid (70% H<sub>3</sub>PO<sub>4</sub>)/liter,

50.0% H<sub>2</sub>O

7. A relatively stable multiple action lubricating composition for application to a steel work piece substan-

## 12

tially of ferritic crystal structure, to provide on the work piece both a chemically deposited coating capable of providing a high degree of separation of work and tool during said working of the piece and an organic friction reducing substance, said composition consisting of:

7.0% oleic acid,

3.0% stearic acid,

16.5% of an organic amide lubricant having the following molecular composition:

1 mole glycerine mono-fatty acid ester,



2 moles fatty amide,



25.0% of an amide lubricant having the following molecular composition:

1 mole glycerine di-fatty acid ester,



1 mole fatty amide



10.3% condensation product of ethylene oxide and an organic acid

7.2% phosphoric acid (70% H<sub>3</sub>PO<sub>4</sub>),

30 31.0% of an acid zinc phosphate solution containing 178 grams zinc/liter and 1200 grams phosphoric acid (70% H<sub>3</sub>PO<sub>4</sub>)/liter,

where RCO— and



each represent the acyl radicals of mixed saturated and mono-unsaturated fatty acids of 16 and 18 carbon atoms.

## References Cited in the file of this patent

## UNITED STATES PATENTS

|           |                 |               |
|-----------|-----------------|---------------|
| 1,007,069 | Coslett         | Oct. 31, 1911 |
| 1,888,189 | Tanner et al.   | Nov. 15, 1932 |
| 1,925,305 | Cohn            | Sept. 5, 1933 |
| 1,949,090 | Tanner et al.   | Feb. 27, 1934 |
| 2,008,939 | Tufts           | July 23, 1935 |
| 2,105,015 | Singer          | Jan. 11, 1938 |
| 2,328,540 | Hochwalt        | Sept. 7, 1943 |
| 2,333,206 | Sloan           | Nov. 2, 1943  |
| 2,385,800 | Douty et al.    | Oct. 2, 1945  |
| 2,403,426 | Douty et al.    | July 2, 1946  |
| 2,470,136 | Bramberry       | May 17, 1949  |
| 2,472,393 | Avallone et al. | June 7, 1949  |

## FOREIGN PATENTS

|         |               |               |
|---------|---------------|---------------|
| 496,866 | Great Britain | Dec. 7, 1933  |
| 697,556 | Germany       | Oct. 17, 1940 |
| 70,135  | Norway        | Nov. 28, 1944 |